

Aug. 15, 1933.

**C. R. SHORT**

1,922,402

## METHOD OF SINTERING BRIQUETTED MATERIALS

Filed Feb. 24, 1930.



Inventor

Charles R. Short

By Spencer Hardman & Fehr

## UNITED STATES PATENT OFFICE

1,922,402

## METHOD OF SINTERING BRIQUETTED MATERIALS

Charles R. Short, Dayton, Ohio, assignor to  
Moraine Products Company, Dayton, Ohio, a  
Corporation of Ohio

Application February 24, 1930. Serial No. 430,834

6 Claims. (Cl. 75—1)

This invention relates to the art of heat-treating or sintering metal structures such as briquetted metal powders.

As disclosed in Patent 1,642,348 to Williams et al, issued Sept. 13, 1927, finely divided metals such as copper, tin and zinc and a volatile fluxing material have heretofore been mixed together in various combinations and proportions according to the desired characteristics of the product. The mixture may also include finely divided graphite and volatile void-forming substances, especially when greater porosity is desired. The mixture is briquetted under high pressure to form the bearing bushings, or any other desired article, and then the briquettes are sintered under conditions to cause the metals to cohere, diffuse or alloy in order to form a strongly coherent metal structure. One known method of sintering is to place the briquettes in a suitable metal box and pack charcoal or bonite around the briquettes and cover the box with a loose fitting cover. The box and contents are heated in a furnace chamber for a determined period to sinter the metals together and are then removed and cooled down. Oxidation of the metal constituents of the briquettes is prevented by the enveloping charcoal bed. Instead of sintering in packed charcoal boxes, the briquettes may be immersed in a fluxing liquid which is also the heating medium, for example, molten potassium cyanide. Of course, when so immersed, all oxidation of the briquettes is prevented.

The present invention has for an object to provide a novel method of sintering such briquettes which is very much more rapid and economical than prior methods and which produces sintered bodies having greater strength and greater uniformity in physical properties.

Further objects and advantages of the present invention will be apparent from the following description, reference being had to the accompanying drawing wherein a preferred embodiment of one form of the present invention is clearly shown.

## 45 In the drawing:

Fig. 1 is a longitudinal vertical section through a continuous sintering furnace for carrying out the methods of this invention.

Fig. 2 is a transverse section on line 2—2 of Fig. 1.

Fig. 3 is a detail view taken on line 3—3 of Fig. 2 and illustrates the direct contact of the pyrometer element with the briquette container when said container is being rapidly heated in the quick-heating chamber of the furnace.

Similar reference characters refer to similar parts throughout the various views.

The furnace comprises a quick-heating chamber 10 and a main sintering chamber 11, both of which are enclosed by suitable heat retaining

walls 12. A continuous track 15 extends entirely through both chambers 10 and 11 and projects out at 16 at the entrance opening 20 of the furnace and at 17 at the exit opening 21 thereof. The wall 22 dividing chambers 10 and 11 is provided with an opening 25 which is sufficiently large for the briquette containers 26 to easily pass therethrough along the track 15. Both chambers 10 and 11 have a false bottom wall 13 therein, under which are the regulated gas burners or outlets 18 and 19. The burners 18 supply heat to the quick heating chambers 10 and are separately regulated from the burners 19 which supply heat to the sintering chamber 11. By this means the entrance chamber 10 is maintained at a substantially higher temperature than the sintering chamber 11, whereby each container 26 of briquettes 30 on entering the furnace is quickly heated to the desired temperature before it is passed on into the sintering chamber 11 which is maintained at the desired sintering temperature.

In the operation of the furnace, a large number of closed containers 26 is provided. These containers are loaded with an equal weight of the briquettes 30. The filled containers 26 are then set upon the projecting track 16 and pushed one at a time into the quick-heating chamber 10, which is large enough to accommodate at least two containers 26 so that while the first container in position "B" is approaching sintering temperature, the second receives a preliminary heating in position "A". An important feature of the invention is the direct measuring of the temperature of the container 26 during its quick heating so that each container is heated quickly to an accurately controlled predetermined temperature before it is passed on into the sintering chamber 11. For directly measuring the temperature of the container 26 while it is being rapidly heated to, or approximately to the desired sintering temperature, a pyrometer element 35 is pivotally mounted at 36 and weighted by a weight 37 so that its thermo-couple 38 will be urged upwardly and contact directly upon the bottom of each container 26 when it is in position "B" (see Fig. 1). The electric wires 39 of the pyrometer lead to a visible temperature indicating, and also preferably recording, device in easy view of the operator.

When the operator notes that the container 26 in position "B" has reached the desired predetermined temperature he immediately pushes it along track 15 through the opening 25 into the main sintering chamber 11. Ordinarily this is done by placing a newly filled container 26 on the projecting track portion 16 and by means of a suitable rod pushing the entire line of containers a distance of one position. This of course will eject the last container 26 through the exit opening 21 of chamber 11, and move the con-

tainer in chamber 10 from position A to position B.

As one example of the material of the briquettes 30 the following is given:

|                   | Parts |
|-------------------|-------|
| Copper powder     | 90    |
| Tin powder        | 10    |
| Salicylic acid    | 6     |
| Ammonium chloride | 0.53  |

10 These materials are briquetted into the form of bearing bushings under high pressure as disclosed in above mentioned Patent No. 1,642,348, forming the briquettes 30 of the above description. In the furnace illustrated the quick-heating chamber 10 accommodates two containers and may be heated to a temperature of 1700° F., and the sintering chamber 11 accommodates six containers and may be heated to a sintering temperature of 1500° F. When the container in position "B" in chamber 10 is heated to nearly the desired sintering temperature, say 1450° F., as indicated by the pyrometer, it is pushed into the sintering chamber 11. It is preferred to heat the briquettes in chamber 10 from room temperature to sintering temperature as rapidly as possible consistent with substantially uniform heating of all the briquettes in a container since it is found that the strength of the sintered bearing is greatly increased by such rapid heating. If now it requires six minutes to heat the containers from room temperature to 1450° F., a container will be pushed from chamber 10 into chamber 11 every three minutes. Now since there are six positions in chamber 11, each container will remain therein for 18 minutes, during which time sintering of the powdered materials of the briquettes takes place. The ammonium chloride therein volatilizes during sintering and fills the containers 26 40 with a gaseous flux which also of course ejects the air from said containers at the crevices around the covers and so provides a non-oxidizing atmosphere therein.

45 The actual time required in the chambers of the furnace will vary chiefly according to the weight and shape of the briquettes; for instance, if the briquettes have a thick heavy portion they obviously cannot be heated so rapidly in chamber 10. A very important feature of the method of this invention is the substantially exact temperature control of the material in the container 26 in position "B" in chamber 10 whereby the highly desirable uniformity of the sintered bushings is obtained. Heretofore standard practice in heat-treating furnaces is to maintain the furnace chamber at a given temperature and to move the articles being heat-treated therethrough on a time cycle. Obviously this method will not fix or control the exact temperature of the article being treated, especially if there is any variation in the size or thickness of the articles. The method of this invention does not rely on a time cycle at all, but proceeds by measuring directly the fundamental factor in the heat treatment of the material, that is the temperature of the article itself.

55 While the form of embodiment of the present invention as herein disclosed constitutes a preferred form, it is to be understood that other forms may be adopted, all coming within the scope of the claims which follow.

60 What is claimed is as follows:

1. The method of sintering articles briquetted from finely divided metals, comprising: rapidly heating the articles to a temperature near a pre-

determined sintering temperature by exposing them to a temperature higher than said sintering temperature, and then substantially immediately passing said heated articles into a sintering zone where they are maintained at the sintering temperature until sintered.

80

2. The method of sintering articles briquetted from finely divided metals, comprising: heating the articles substantially as rapidly as possible consistent with the uniform heating of said articles to a temperature near a predetermined sintering temperature by exposing said articles to a temperature higher than said sintering temperature, and then quickly passing said heated articles into a sintering zone maintained at the sintering temperature and permitting said articles to remain in said sintering zone until sintering is completed.

85

3. The method of sintering highly compressed briquettes of finely divided metals such as copper, tin and zinc, comprising: heating the briquettes to a predetermined temperature near the desired sintering temperature at a high rate of temperature change by exposing the briquettes to a temperature higher than the sintering temperature, measuring the temperature of said briquettes as distinguished from the temperature of the chamber in which they are heated to avoid heating the briquettes beyond said sintering temperatures, and upon said predetermined temperature being reached thereafter substantially immediately exposing said briquettes to the sintering temperature for a period of time until the metal powders are sintered together.

95

4. The method of sintering articles of briquetted metal powders, comprising: exposing a plurality of articles in a thin wall metal container to a temperature considerably hotter than the desired predetermined sintering temperature, directly measuring the temperature of said container as it rapidly rises due to such heating and when said container approaches said sintering temperature, passing it quickly into a sintering zone maintained at the desired sintering temperature where sintering occurs for a period of time.

100

5. The method of sintering articles briquetted from finely divided metals, comprising: inserting a plurality of said articles in a thin wall metal container and then heating said container and articles therein substantially as rapidly as possible consistent with the substantially uniform heating of said articles by exposing them to a temperature higher than a predetermined sintering temperature until the temperature of the articles approaches said sintering temperature, and then quickly passing said heated container and articles therein into a sintering zone maintained at said sintering temperature and permitting said articles to remain therein until sintering is completed.

105

6. The method of sintering articles briquetted from finely divided metals, comprising: first rapidly heating the articles to a temperature near a predetermined sintering temperature in a quick-heating zone having such a high rate of heat supply thereto that said articles would be quickly heated beyond said sintering temperature if they remained therein after reaching said sintering temperature, then substantially immediately passing said heated articles into a sintering zone maintained at said predetermined sintering temperature and permitting said articles to remain therein until sintering is completed.

110